

June 18, 1957

R. I. JAFFEE ET AL

2,796,347

TITANIUM BASE ALLOYS CONTAINING ANTIMONY

Filed Nov. 23, 1953

COMPARATIVE STRENGTHENING  
EFFECTS OF Al, Sb AND Sn ALLOY  
ADDITIONS TO COMMERCIAL  
PURITY Ti-BASE



INVENTORS.  
ROBERT I. JAFFEE.  
HORACE R. OGDEN.  
BY RALPH A. HAPPE.

Ward Crosby & Neal.  
ATTORNEYS.

**1**

2,796,347

**TITANIUM BASE ALLOYS CONTAINING ANTIMONY**

Robert I. Jaffee, Worthington, and Horace R. Ogden, Columbus, Ohio, and Ralph A. Happe, Anaheim, Calif., assignors, by mesme assignments, to Rem-Cru Titanium Incorporated, Midland, Pa., a corporation of Pennsylvania

Application November 23, 1953, Serial No. 393,578

12 Claims. (Cl. 75—175.5)

This invention pertains to binary alloys of titanium and antimony and also to ternary and higher component alloys formed therewith by additions of other elements including alpha-promoting, beta-promoting and compound-forming elements.

This application is a continuation-in-part of our co-pending applications Serial No. 327,421, filed December 22, 1952, and Serial No. 371,112, filed July 29, 1953, now abandoned.

The alloys of the invention are in general characterized by excellent mechanical properties, possessing high tensile strength as compared to the unalloyed titanium-base metal, combined with adequate ductility for both hot and cold forming operations, i. e., forging, rolling, etc. The binary alloys of the invention may be welded without appreciable loss of ductility in the welded as compared to non-welded portions. And the same is generally true of the ternary and higher component alloys as shown by the test data set forth below. The alloys of the invention also have good contamination resistance as regards oxidation and penetration by atmospheric gases at room and elevated temperatures.

The binary titanium-base alloys of the invention are quite ductile throughout the range of about 1 to 18% Sb. Higher antimony additions result in increasing brittleness, but are useful in cast form for antimony additions up to about 25%. The ductile Ti—(1-18%)Sb base alloys are greatly strengthened without appreciable loss of ductility by additions of limited and controlled amounts of the interstitials, carbon, oxygen and nitrogen. To this end, carbon may be present up to about 0.6%, oxygen up to about 0.4% and nitrogen up to about 0.3%. Further strengthening with retention of adequate ductility results from additions of other elements, including alpha-promoters, beta-promoters and compound-forming elements, as enumerated and in proportions as set forth

**2**

below, the lower the antimony content the higher the tolerance for such additions and vice versa.

As is known, the metal titanium in the pure state, is capable of existing in either of two allotropic forms. Below a temperature of about 885° C. or 1625° F., it assumes a close-packed hexagonal structure known as the alpha phase, while at this temperature and above it assumes a body-centered cubic structure known as the beta phase.

Certain substitutional alloying additions to the titanium-base metal, among which may be mentioned aluminum, indium, bismuth and lead, as well as the interstitials carbon, oxygen and nitrogen, tend to stabilize the alpha phase.

Our investigations with iodide-base titanium-antimony alloys have shown that antimony has a slight beta stabilizing tendency in that the transformation range shifts progressively downward to about 840° C. as the antimony content is increased to the terminal alpha solubility of about 17.5%. It should be emphasized, however, that antimony has thus a relatively indifferent effect on the transformation temperature of titanium. It produces all-alpha alloys with titanium which undergo no hardening on quenching from the beta field. Antimony may thus be considered an alpha stabilizer, and it will be so treated in the following.

Tin behaves in a manner quite analogous to antimony and likewise should be treated as an alpha stabilizer. Silver, formerly considered an alpha stabilizer, now appears more properly grouped similarly to tin and antimony.

30 The effect of silver on the transformation range is so slight that silver may be considered as either an alpha or beta stabilizer, and it will be treated as an alpha stabilizer in the following.

Other substitutional alloying elements, when added in progressively increasing quantities, stabilize the beta phase at progressively lower temperatures, until a mixed alpha-beta or stable all-beta microstructure is obtained at normal or atmospheric temperatures, or the beta phase undergoes a eutectoid reaction, depending on the character and amount of the beta stabilizers added.

Speaking in broadest terms, the beta stabilizers are Mo, V, Cb, Ta, Zr, Mn, Fe, Cr, W, Co, Ni and Cu. Silicon and beryllium may also be considered as beta stabilizing elements, but their solubilities in titanium are relatively small, so that it is equally proper to consider them as compound-forming elements. Within this broad category, however, only certain of the elements mentioned are suitable for producing mixed-phase, alpha-beta alloys, or all-beta alloys. These are the elements which have beta-iso-

morphous diagrams, or which have beta-eutectoid diagrams such that the decomposition of the beta phase into eutectoid is so sluggish that the alloys behave like those in a beta-isomorphous system. The beta stabilizing elements of this type are Mo, V, Cb, Ta, Mn, Fe, Cr and W. Within this group only Mo, V, Cb and Ta are beta-isomorphous. They form the most thermally stable beta-containing alloys, as a result of their beta-isomorphism.

Zirconium is a beta promoter or stabilizer in the sense that the lowest temperature at which alloys thereof with titanium are entirely beta, becomes progressively lower with increasing amounts of zirconium, until a composition is reached at which this so-called beta transus temperature starts to increase again with further additions of zirconium. While zirconium thus lowers the transformation temperature of titanium, the alloys eventually revert to the alpha phase at lower temperatures unless other beta-promoters are present. Zirconium is isomorphous with titanium both in the alpha and beta fields. As a result, it is proper to consider zirconium together with vanadium, molybdenum, columbium and tantalum as all being beta-isomorphous with titanium.

The use of copper alone as an alloying addition to titanium, does not fit into the above-mentioned grouping of beta-isomorphous and sluggishly decomposing eutectoid beta promoters, because the beta phase stabilized by copper always decomposes rather rapidly into pro-eutectoid and eutectoid products, and the same is generally true with respect to cobalt, nickel, silicon and beryllium, above listed under the broad category of beta stabilizers. Copper, however, is a useful addition when present as a minor alloying element, for example, up to a few percent, in alloys containing larger amounts of other beta-stabilizing elements, within the limited group of beta-promoters last mentioned above since, in these low concentrations and in the presence of such other beta-stabilizing elements, the tendency of the beta phase stabilized in part by copper to decompose into eutectoid products is minimized or entirely eliminated.

The tolerance of the Ti—Sb base alloys of the invention with respect to additions of the various beta-promoters above mentioned, varies considerably for the individual elements of this group, being greatest with respect to those which form beta-isomorphous systems with titanium, and least for those which decompose most readily into eutectoid decomposition products. Thus, the Ti—Sb base alloys may be strengthened without undue embrittlement by additions of up to about 40% or even up to 50% in aggregate of elements composing the beta-isomorphous group, viz., molybdenum, vanadium, columbium, tantalum and zirconium. Of the sluggishly decomposing elements, the base alloy will tolerate additions of up to about 25% of either or both chromium and tungsten, up to about 10% manganese, and up to about 7% iron. Metal of the group cobalt, nickel and copper may be added up to a total of about 5%. For additions of all of the above-mentioned beta-promoters, the lower effective limit is about 0.5% and preferably about 1%. In all of the alloys in this category, the antimony content should be on the low side of its range when the beta-promoter addition is on the high side of its range and vice versa.

The tolerance of the Ti—Sb base alloys for the alpha promoters depends on the amount of antimony present, the less antimony present the greater the amount of alpha-promoters that can be added, and vice versa. Aluminum may be added to a maximum content of 8%, and tin may be added to a maximum content of 22.5%. The proportioning of aluminum at the high antimony contents and of tin are given subsequently. Indium and silver may be added up to a maximum content of 15%. Lead and bismuth may be added up to 15% added to the charge in melting.

The elements Ce, B, As, S, Te and P are strictly com-

pound-forming elements. They do not have appreciable solubilities in either the alpha or beta phase, but form intermetallic compounds with titanium. The beta promoters silicon and beryllium are likewise best grouped as compound-forming elements, in view of their above-mentioned low solubilities in titanium. The Ti—Sb alloys of the invention will tolerate only relatively small amounts of these compound-forming elements, i. e., up to a total of about 2% maximum, the lower effective limit being about 0.1 or 0.2%.

Substantially pure and ductile metallic titanium may be produced at considerable expense by the so-called "iodide" process described in U. S. Patent 1,671,213 to Van Arkel; while ductile titanium of commercial purity is produced more cheaply by the magnesium reduction of titanium tetrachloride by the process described in U. S. Patent 2,205,854 to Kroll. Both procedures, particularly the latter, result in some contamination of the titanium metal with one or more of the interstitials, carbon, oxygen and nitrogen. But since, as noted above, these are all alpha-promoting or stabilizing elements, the resultant somewhat contaminated titanium metal obtained, has at room temperatures a single phase, all-alpha microstructure.

The all-alpha, all-beta and mixed alpha-beta alloys of titanium have their respective advantages and disadvantages. Generally speaking, the alpha alloys provide good all around performance, having good weldability, and being strong and resistant to oxidation, both cold and hot, but are somewhat inferior as to ductility. The all-beta alloys, on the other hand, have excellent bendability and ductility, are strong both hot and cold, but are somewhat vulnerable to atmospheric contamination, particularly at elevated temperatures. The mixed alpha-beta alloys provide a compromise performance as between all-alpha and all-beta alloys, being strong when cold and warm, but weak hot, while possessing good bendability and ductility, with a moderate degree of resistance to atmospheric contamination.

The following Table I gives the mechanical properties of the binary alloys of antimony and iodide-base titanium over the ductile range of about 1-18% Sb. The succeeding Table II gives the corresponding values for the binary alloys of antimony and titanium-base metal of commercial purity. This table also shows the strengthening effect of additions of the interstitials carbon, oxygen and nitrogen.

Referring to Table I, it will be seen that additions of up to about 18% antimony to iodide-base titanium more than trebles the yield strength and approximately trebles the ultimate strength with retention of adequate ductility for fabrication purposes. The yield strength increases from 24,000 p. s. i. to upwards of 80,000 p. s. i., and the ultimate strength increases from 40,000 to about 100,000 p. s. i., while retaining the minimum bend ductility at values under 4T, and the percent tensile elongation at values of upwards of about 15%.

Referring to Table II, for the commercial purity titanium-base values, the yield strength is more than doubled by additions of antimony up to about 18%, the yield strength increasing from about 48,000 to about 110,000 p. s. i., and the ultimate strength from about 71,000 to about 120,000 p. s. i. As further shown by the test data, the binary alloys become somewhat embrittled above about 16% Sb, although they can still be fabricated. Additions of the interstitials further enhance the tensile properties while reducing the ductility but slightly. Thus with the Ti—10% Sb alloy, the addition of up to 0.4% carbon approximately doubles both the yield and ultimate strengths from 77,000 to 147,000 and from 91,000 to 148,000 p. s. i., respectively. Also as shown by the comparison of values for additions of 0.2% each of carbon, oxygen and nitrogen, oxygen has a slightly inferior strengthening effect as compared to carbon, while nitrogen has a somewhat greater strengthening effect than carbon.

TABLE I  
*Mechanical properties of iodide titanium-base Ti—Sb alloys*

[These alloys were 980° C. forged, 850° C. rolled to 0.04" and annealed 2 hours at 850° C. and air cooled]

| Composition,<br>Percent<br>(Balance<br>Titanium) | Tensile properties:<br>p. s. i. $\times 1,000$ |                      | Percent<br>Elonga-<br>tion<br>in 1" | Percent<br>Reduction<br>in Area | Vickers<br>Hardness | MBR, T<br>Annealed |     | MBR, T<br>Aged 48<br>Hours<br>at 400°<br>C. L. |
|--------------------------------------------------|------------------------------------------------|----------------------|-------------------------------------|---------------------------------|---------------------|--------------------|-----|------------------------------------------------|
|                                                  | 0.2%<br>Offset<br>Yield                        | Ultimate<br>Strength |                                     |                                 |                     | L                  | T   |                                                |
| 100Ti                                            | 24                                             | 40                   | 53                                  | 54                              | 102                 | 0                  | 0   | -----                                          |
| 2.5Sb                                            | 25                                             | 42                   | 39                                  | 71                              | 117                 | 0                  | 0   | -----                                          |
| 5Sb                                              | 32                                             | 49                   | 30                                  | 60                              | 135                 | 0.6                | 1.1 | 0.6                                            |
| 7.5Sb                                            | 42                                             | 62                   | 28                                  | 54                              | 180                 | 1.6                | 1.7 | 1.9                                            |
| 10Sb                                             | 54                                             | 68                   | 18                                  | 53                              | 198                 | 1.9                | 1.9 | 2.5                                            |
| 12.5Sb                                           | 66                                             | 78                   | 20                                  | 49                              | 222                 | 2.4                | 2.3 | 2.3                                            |
| 15Sb                                             | 86                                             | 103                  | 15                                  | 39                              | 254                 | 3.4                | 3.2 | 1.6                                            |
| 17.5Sb                                           | 82                                             | 98                   | 14                                  | 38                              | 255                 | 3.7                | 3.2 | -----                                          |
| 20Sb                                             | (1)                                            | (1)                  | (1)                                 | (1)                             | (1)                 | (1)                | (1) | (1)                                            |

<sup>1</sup> Could not be fabricated.

TABLE II

*Mechanical properties of commercial purity titanium-base Ti—Sb alloys*

[These alloys were 980° C. forged, 850° C. rolled and annealed 2 hours at 850° C.]

| Composition, Percent<br>(Balance Titanium) | Tensile Properties:<br>p. s. i. $\times 1,000$ |                      | Percent<br>Elonga-<br>tion<br>in 1" | Percent<br>Reduction<br>in Area | VHN | MBR, T |     | T |
|--------------------------------------------|------------------------------------------------|----------------------|-------------------------------------|---------------------------------|-----|--------|-----|---|
|                                            | 0.2%<br>Offset<br>Yield                        | Ultimate<br>Strength |                                     |                                 |     | L      | T   |   |
| 100Ti                                      | 48                                             | 71                   | 21                                  | 51                              | 187 | 0.8    | 0.8 |   |
| 1Sb                                        | 48                                             | 72                   | 25                                  | 49                              | 179 | 0.4    | 1.2 |   |
| 2.5Sb                                      | 51                                             | 75                   | 25                                  | 49                              | 202 | 1.2    | 1.6 |   |
| 5Sb                                        | 58                                             | 77                   | 22                                  | 47                              | 227 | 1.5    | 1.6 |   |
| 7.5Sb                                      | 71                                             | 86                   | 20                                  | 49                              | 257 | 1.8    | 2.8 |   |
| 10Sb                                       | 77                                             | 91                   | 19                                  | 46                              | 267 | 1.5    | 1.6 |   |
| 12.5Sb                                     | 90                                             | 101                  | 11                                  | 48                              | 277 | 2.6    | 2.6 |   |
| 15Sb                                       | 99                                             | 111                  | 15                                  | 43                              | 304 | 2.5    | 2.5 |   |
| 16Sb                                       | 114                                            | 118                  | 10                                  | 31                              | 331 | 2.5    | 6.4 |   |
| 17Sb                                       | 115                                            | 124                  | 12                                  | 32                              | 322 | Br     | 7.0 |   |
| 18Sb                                       | 109                                            | 118                  | 4                                   | 14                              | 330 | Br     | Br  |   |
| 19Sb                                       | (1)                                            | (1)                  | (1)                                 | (1)                             | (1) | (1)    | (1) |   |
| 10Sb-0.2C                                  | 124                                            | 125                  | 8                                   | 43                              | 348 | 1.5    | 2.4 |   |
| 10Sb-0.4C                                  | 147                                            | 148                  | 17                                  | 42                              | 388 | 3.0    | 4.7 |   |
| 10Sb-0.2O                                  | 113                                            | 120                  | 16                                  | 40                              | 346 | 2.5    | 5.0 |   |
| 10Sb-0.2N                                  | 131                                            | 134                  | 15                                  | 42                              | 369 | 2.4    | 4.8 |   |

<sup>1</sup> Could not be fabricated.

In U. S. Patent 2,596,487, granted May 13, 1952, to Jaffee, Ogden and Maykuth as joint inventors, there is described a series of titanium-aluminum base alloys containing 3.5 to 5% Al, the properties of which are improved by additions of 0.5 to 5.0% antimony together with 0.02 to 0.3% and preferably about 0.25% carbon. The present applicants have discovered in accordance with one aspect of the present invention, that strong and ductile alloys result from additions of about 0.25 to 5% and preferably about 0.25 to under 3.5% of aluminum to titanium-antimony base alloys containing from more than 5% and preferably from about 6% to about 18% antimony, the antimony being on the low side when aluminum is on the high side of the aforesaid ranges and vice versa. The preferred maximum antimony content for a

given aluminum content is shown by the following relationship:

| Percent<br>Aluminum | Percent<br>Antimony,<br>Max. |
|---------------------|------------------------------|
| 0.25                | 18.0                         |
| 1.0                 | 16.0                         |
| 2.0                 | 14.0                         |
| 3.0                 | 12.5                         |
| 4.0                 | 11.0                         |
| 5.0                 | 10.0                         |

The foregoing conclusions are based on the test results given in the following Table III, showing the effect of

additions of this important alpha promoter, aluminum, to the Ti—Sb base alloys of the invention. This data clearly establishes that additions of aluminum have a tremendous strengthening effect on the Ti—Sb base alloy. Thus, for example, the addition of as little as 1% aluminum to the Ti—5% Sb alloy increases the yield strength by about 40% and the ultimate strength by about 20%, or from 48,000 to 80,000 p. s. i. for the yield strength and from

5 purity base alloys of Table II are plotted against the antimony content, and the same is done for the Ti—Al commercial purity binaries, as shown in the accompanying drawing, it will be found that to a close degree of approximation, 1% of aluminum is equivalent to about 3% of either antimony or tin, as regards strengthening effect. The data in Table III illustrates that this equivalency holds approximately in ternary Ti—Al—Sb alloys.

TABLE III  
Mechanical properties of Ti—Sb—Al alloys (commercial purity Ti-base)

[These alloys were 980° C. forged, 850° C. rolled and annealed 2 hours at 850° C.]

| Composition, Percent<br>(Balance Titanium) | Tensile Properties:<br>p. s. i. $\times 1,000$ |                      | Percent<br>Elonga-<br>tion in 1" | Percent<br>Reduc-<br>tion in<br>Area | Vickers<br>Hardness | MBR, T |     |
|--------------------------------------------|------------------------------------------------|----------------------|----------------------------------|--------------------------------------|---------------------|--------|-----|
|                                            | 0.2% Off-<br>set Yield                         | Ultimate<br>Strength |                                  |                                      |                     | L      | T   |
| 100Ti                                      | 53                                             | 77                   | 22                               | 50                                   | 202                 | 0.7    | 1.8 |
| 4Sb—4Al                                    | 112                                            | 120                  | 15                               | 32                                   | 345                 | 2.4    | 3.1 |
| 5Sb—4Al                                    | 110                                            | 115                  | 20                               | 46                                   | 351                 | 2.7    | 2.7 |
| 6Sb—4Al                                    | 118                                            | 124                  | 17                               | 33                                   | 352                 | 3.5    | 3.4 |
| 6Sb—4Al                                    | 121                                            | 126                  | 15                               | 39                                   | 355                 | 3.4    | 2.5 |
| 7Sb—4Al                                    | 120                                            | 122                  | 15                               | 44                                   | 360                 | 3.5    | 2.6 |
| 5Sb—1Al                                    | 58                                             | 77                   | 22                               | 47                                   | 227                 | 1.5    | 1.6 |
| 5Sb—2Al                                    | 80                                             | 91                   | 16                               | 42                                   | 262                 | 2.1    | 2.2 |
| 5Sb—3Al                                    | 92                                             | 96                   | 12                               | 46                                   | 288                 | 1.5    | 2.0 |
| 5Sb—3Al                                    | 96                                             | 102                  | 15                               | 49                                   | 311                 | 2.1    | 2.1 |
| 6Sb—3Al                                    | 104                                            | 111                  | 19                               | 46                                   | 323                 | 2.8    | 2.6 |
| 6Sb—4Al                                    | 118                                            | 124                  | 17                               | 33                                   | 352                 | 3.5    | 3.4 |
| 6Sb—4Al                                    | 121                                            | 126                  | 15                               | 39                                   | 355                 | 3.4    | 2.5 |
| 6Sb—5Al                                    | 128                                            | 129                  | 15                               | 40                                   | 336                 | 5.0    | 3.3 |
| 7.5Sb                                      | 71                                             | 86                   | 20                               | 49                                   | 257                 | 1.8    | 2.8 |
| 7.5Sb—4Al                                  | 121                                            | 124                  | 16                               | 39                                   | 356                 | 2.8    | 3.8 |
| 10Sb                                       | 77                                             | 91                   | 19                               | 46                                   | 267                 | 1.5    | 1.6 |
| 10Sb—1Al                                   | 104                                            | 108                  | 18                               | 48                                   | 298                 | 2.1    | 1.9 |
| 10Sb—2Al                                   | 119                                            | 121                  | 12                               | 43                                   | 342                 | 2.5    | 3.1 |
| 10Sb—3Al                                   | 128                                            | 132                  | 9                                | 37                                   | 350                 | 2.8    | 3.6 |
| 10Sb—4Al                                   | 130                                            | 131                  | 13                               | 28                                   | 376                 | 2.5    | —   |
| 10Sb—5Al                                   | 144                                            | 144                  | 8                                | 29                                   | 356                 | —      | Br  |
| 12.5Sb                                     | 90                                             | 101                  | 11                               | 48                                   | 277                 | 2.6    | 2.6 |
| 12.5Sb—1Al                                 | 114                                            | 120                  | 20                               | 41                                   | 312                 | 2.1    | 4.0 |
| 12.5Sb—2Al                                 | 128                                            | 128                  | 8                                | 38                                   | 353                 | 2.3    | 4.9 |
| 12.5Sb—3Al                                 | 135                                            | 138                  | 6                                | 28                                   | 355                 | Br     | Br  |
| 12.5Sb—4Al                                 | (1)                                            | (1)                  | (1)                              | (1)                                  | (1)                 | (1)    | (1) |
| 15Sb                                       | 99                                             | 111                  | 15                               | 43                                   | 304                 | 2.5    | 2.5 |
| 15Sb—1Al                                   | 127                                            | 131                  | 12                               | 46                                   | 342                 | 3.1    | 3.8 |
| 15Sb—2Al                                   | 139                                            | 142                  | 8                                | 37                                   | 345                 | Br     | 5.3 |
| 15Sb—3Al                                   | (2)                                            | (2)                  | (2)                              | (2)                                  | (2)                 | (2)    | (2) |
| 17Sb                                       | 115                                            | 124                  | 12                               | 32                                   | 322                 | Br     | 7.0 |
| 17.5Sb—1Al                                 | 140                                            | 144                  | 5                                | 27                                   | 338                 | Br     | —   |
| 17.5Sb—2Al                                 | (1)                                            | (1)                  | (1)                              | (1)                                  | (1)                 | (1)    | (1) |

<sup>1</sup> Could not be fabricated.

<sup>2</sup> Too brittle for testing.

77,000 to 91,000 p. s. i. for the ultimate strength, without impairing the ductility in any appreciable degree, the minimum bend ductility being about 2.2 T and the percent tensile elongation about 16%. Further strengthening of the Ti—5% Sb alloy results from additions of up to 3% aluminum, the yield strength being thus increased to 96,000 and the ultimate strength to 120,000 p. s. i., while still retaining substantially the same ductility, i. e., about 2 T for the minimum bend and about 15% for tensile elongation. Corresponding enhancements in tensile strength with retention of adequate ductility result from additions of up to 4% Al to the Ti—10% Sb base alloy, the yield strength increasing from 77,000 to 130,000 p. s. i. and the ultimate strength from 91,000 to 131,000 p. s. i., the minimum bend increasing to only 2.5 T. About the same strengthening enhancements result from additions of up to about 3% Al to the 12.5% Sb base alloy, and up to about 2% Al to the 15% Sb base alloy, and up to about 1% Al for the 17.5% Sb base alloy, consistent with retention of adequate ductility for purposes of fabrication.

If the tensile properties for the Ti—Sb, commercial

55 As shown in the copending joint application of W. L. Finlay and the applicants Jaffee and Ogden herein, Serial No. 341,796, filed March 11, 1953, the upper limit for additions of tin to titanium which can be fabricated, is about 23%. Correspondingly, it is shown in the present application that the upper limit for additions of antimony to titanium which can be fabricated, is about 18%. The following Table IV gives test data establishing the upper limit for combinations of titanium, tin and antimony. Thus from the data of Table IV, it will be seen that the maximum amount of tin that may thus be added to the 60 Ti—Sb base alloy, for any given percentage of antimony present, is as set forth in the following tabulation:

| Percent<br>Antimony | Percent<br>Tin, Max. |
|---------------------|----------------------|
| 18                  | 0                    |
| 15                  | 5                    |
| 10                  | 12.5                 |
| 5                   | 17.5                 |
| 0.5                 | 22.5                 |

TABLE IV  
*Mechanical properties of Ti—Sb—Sn and  
 Ti—Sb—Sn—Al alloys.*

(Commercial purity Ti-bases)

[These alloys were 980° C. forged, 850° C. rolled and annealed two hours at 850° C.]

| Composition, percent (Balance<br>Titanium) | Tensile Properties:<br>p. s. i. $\times 1,000$ |                      | Percent<br>Elonga-<br>tion<br>in 1" | Percent<br>Reduction<br>in<br>Area | Vickers<br>Hard-<br>ness | MBR, T |         |
|--------------------------------------------|------------------------------------------------|----------------------|-------------------------------------|------------------------------------|--------------------------|--------|---------|
|                                            | 0.2% Off-<br>set Yield                         | Ultimate<br>Strength |                                     |                                    |                          | L      | T       |
| 5Sb—                                       | 58                                             | 77                   | 22                                  | 47                                 | 227                      | 1.5    | 1.6     |
| 5Sb—5Sn                                    | 74                                             | 94                   | 17                                  | 46                                 | 262                      | 1.5    | 4.7     |
| 5Sb—10Sn                                   | 100                                            | 111                  | 17                                  | 44                                 | 317                      | 2.5    | 3.2     |
| 5Sb—15Sn                                   | 129                                            | 131                  | 15                                  | 46                                 | 330                      | 2.0    | 3.7     |
| 5Sb—17.5Sn                                 |                                                | 134                  | 0                                   | 6                                  | 338                      |        | 5.2     |
| 6Sb—20Sn                                   | (1)                                            | (1)                  | (1)                                 | (1)                                | (1)                      | (1)    | (1)     |
| 10Sb—                                      | 77                                             | 91                   | 19                                  | 46                                 | 267                      | 2.5    | 2.5     |
| 10Sb—5Sn                                   | 100                                            | 111                  | 17                                  | 44                                 | 317                      | 2.5    | 3.2     |
| 10Sb—10Sn                                  | 125                                            | 133                  | 16                                  | 38                                 | 320                      | 4.9    | 4.9     |
| 10Sb—12.5Sn                                |                                                | 108                  | 0                                   | 0                                  | 330                      | Br     | 7.0     |
| 10Sb—15Sn                                  | (1)                                            | (1)                  | (1)                                 | (1)                                | (1)                      | (1)    | (1)     |
| 10Sb—17.5Sn                                | (1)                                            | (1)                  | (1)                                 | (1)                                | (1)                      | (1)    | (1)     |
| 15Sb—                                      | 99                                             | 111                  | 15                                  | 43                                 | 304                      | 2.5    | 3.3     |
| 15Sb—5Sn                                   |                                                | 126                  | 0                                   | 6                                  | 354                      | Br     | Br      |
| 15Sb—7.5Sn                                 | (1)                                            | (1)                  | (1)                                 | (1)                                | (1)                      | (1)    | (1)     |
| 10Sb—                                      | 77                                             | 91                   | 19                                  | 46                                 | 267                      | 1.5    | 1.6     |
| 7.5Sb—2.5Sn                                | 76                                             | 96                   | 16                                  | 46                                 | 268                      | 2.3    | 3.1     |
| 5Sb—5Sn                                    | 74                                             | 94                   | 17                                  | 46                                 | 262                      | 1.5    | 4.7     |
| 2.5Sb—7.5Sn                                | 81                                             | 98                   | 18                                  | 43                                 | 270                      | 2.2    | 3.2     |
| 10Sn—                                      | 77                                             | 92                   | 20                                  | 46                                 | 278                      | 1.7    | 2.1     |
| 15Sn—                                      | 99                                             | 111                  | 15                                  | 43                                 | 304                      | 2.5    | 2.5     |
| 12.5Sb—2.5Sn                               | 109                                            | 117                  | 14                                  | 42                                 | 311                      | 1.9    | 3.7     |
| 10Sb—5Sn                                   | 100                                            | 111                  | 17                                  | 44                                 | 317                      | 2.5    | 3.2     |
| 5Sb—10Sn                                   | 107                                            | 116                  | 17                                  | 39                                 | 325                      | 1.7    | 3.5     |
| 2.5Sb—12.5Sn                               | 109                                            | 118                  | 14                                  | 36                                 | 313                      | 2.9    | 5.5     |
| 15Sn—                                      | 107                                            | 117                  | 16                                  | 45                                 | 348                      | 1.8    | 2.7     |
| 10Sb—2.5Al                                 | 123                                            | 125                  | 13                                  | 38                                 | 361                      | 2.4    | 3.3     |
| 7.5Sb—2.5Sn—2.5Al                          | 110                                            | 115                  | 15                                  | 48                                 | 339                      | 2.6    | 3.4     |
| 5Sb—5Sn—2.5Al                              | 114                                            | 118                  | 13                                  | 44                                 | 343                      | 2.8    | 3.6/5.2 |
| 2.5Sb—7.5Sn—2.5Al                          | 110                                            | 117                  | 15                                  | 40                                 | 345                      | 2.6    | 2.5     |
| 10Sn—2.5Al                                 | 113                                            | 119                  | 20                                  | 43                                 | 345                      | 2.5    | 3.2     |
| 10Sb—2.5Al—0.2C                            | 143                                            | 146                  | 16                                  | 47                                 | 393                      | 2.0    | 2.8/Br  |
| 7.5Sb—2.5Sn—2.5Al—0.2C                     | 136                                            | 137                  | 8                                   | 24                                 | 402                      | 2.8    | 2.7/5.3 |
| 5Sb—5Sn—2.5Al—0.2C                         | 154                                            | 157                  | 5                                   | 18                                 | 400                      | 6.2    | Br      |
| 2.5Sb—7.5Sn—2.5Al—0.2C                     | 144                                            | 146                  | 5                                   | 21                                 | 390                      | 3.0    | 5.2     |
| 10Sn—2.5Al—0.2C                            | 140                                            | 141                  | 6                                   | 29                                 | 395                      | 5.5    | Br      |
| 5Al—2.5Sb                                  | 110                                            | 117                  | 15                                  | 42                                 | 352                      | 2.8    | 2.7/5.3 |
| 5Al—2.5Sb—0.5Sn                            | 103                                            | 109                  | 15                                  | 43                                 | 351                      | 2.8    | 3.7     |
| 5Al—1.5Sb—15Sn                             | 106                                            | 113                  | 15                                  | 37                                 | 346                      | 2.1    | 8.6     |
| 5Al—1.5Sb—1.5Sn                            | 103                                            | 112                  | 17                                  | 46                                 | 343                      | 2.9    | 7.6     |
| 5Al—0.5Sb—25Sn                             | 100                                            | 111                  | 14                                  | 43                                 | 348                      | 2.8    | 2.7     |
| 5Al—2.5Sn                                  | 101                                            | 110                  | 17                                  | 47                                 | 344                      | 2.9    | 2.7     |
| 5Al—2.5Sb—0.2O                             | 128                                            | 134                  | 7                                   | 21                                 | 389                      | 2.8    | 7.6     |
| 5Al—2.5Sb—0.5Sn—0.2C                       | (1)                                            | (1)                  | (1)                                 | (1)                                | (1)                      | (1)    | (1)     |
| 5Al—1.5Sb—15Sn—0.2C                        | 132                                            | 135                  | 17                                  | 42                                 | 394                      | 2.8    | 3.5     |
| 5Al—1.5Sb—1.5Sn—0.2C                       | 131                                            | 135                  | 17                                  | 48                                 | 396                      | 2.8    | 2.8/5.5 |
| 5Al—0.5Sb—25Sn—0.2C                        | 130                                            | 134                  | 7                                   | 28                                 | 391                      | 2.8    | 2.8/5.5 |
| 5Al—2.5Sn—0.2C                             | 134                                            | 135                  | 9                                   | 25                                 | 400                      | 2.8    | 6.8     |

<sup>1</sup> Could not be fabricated.

The data in Table IV also establishes that tin is equivalent in strengthening effect to antimony when substituted therefor on a weight percentage basis, i. e., percent for percent. Thus it will be seen that for the series of alloys starting with Ti—10% Sb, in which Sn is progressively substituted for Sb at values of 2.5, 5, 7.5 and 10%, the yield and ultimate strengths remain substantially constant at about 74,000—77,000 p. s. i. and 92,000—98,000 p. s. i., respectively. Likewise for the corresponding series starting with Ti—15% Sb, the yield and ultimate strengths remain substantially constant at about 100,000—109,000 and 111,000—117,000 p. s. i., respectively.

The data in Table IV thus establishes that a substantially direct equivalency exists between tin and antimony additions for Ti—Sn—Sb alloys. In Ti—Al—(Sb, Sn) alloys the preferred maximum antimony content for given aluminum and tin contents is shown by the following relationship:

| Percent<br>Aluminum | Percent Tin | Percent<br>Antimony,<br>Max. |
|---------------------|-------------|------------------------------|
| 0.25                | 5           | 13                           |
| 1                   | 5           | 11                           |
| 2                   | 5           | 9                            |
| 3                   | 5           | 7.5                          |
| 4                   | 5           | 6                            |
| 5                   | 5           | 5                            |

If the tin content is higher, the maximum antimony content is lower, and vice versa, in accordance with the equivalency between tin and antimony. However, for Ti—Al—(Sb, Sn) alloys without carbon additions, the data indicates a trend toward higher strength when no tin is present in the alloys. This is shown by comparison of the values for the series of alloys starting with Ti—10Sb—2.5Al and ending with Ti—10Sn—2.5Al. For the first alloy of the series containing no tin, the yield and ultimate strengths are 123,000 and 125,000 p. s. i., respectively, while for the remaining or tin substituting alloys of the series, the yield and ultimate strengths are lower, in the range of 110,000—114,000 and 115,000—119,000 p. s. i., respectively. This same holds true for the series commencing with Ti—5Al—2.5Sb in which tin is progressively substituted down to Ti—5Al—2.5Sn. For the first or non-tin containing alloy of the series, the yield and ultimate strengths are 110,000 and 117,000 p. s. i., while for the tin-containing analyses, the corresponding values are 101,000—103,000 and 109,000—113,000 p. s. i., respectively. On the other hand, when carbon is present in these aluminum-containing alloys, there appears to exist a direct equivalency between tin and antimony as shown by the further data in Table IV for the alloy series starting with Ti—10Sn—2.5Al—0.2C and Ti—5Al—2.5Sb—0.2C, respectively.

Although as stated, 1% Al is roughly equivalent to 3% Sb in strengthening effect, the data indicate that the

highest yield strengths for a given total equivalent alloy content in Ti—Sb—Al alloys, are obtained when the antimony-aluminum ratio is 5:1; whereas in the Ti—Sn—Al alloys, the strengthening effects of aluminum and tin are approximately additive based on a 3:1 ratio of equivalency of tin to aluminum. The significance of this is that an extra 5,000–10,000 p. s. i. of tensile strengthening can be obtained by using the 5:1 ratio of antimony to aluminum in ternary Ti—Sb—Al alloys over what can be obtained in the equivalent Ti—Sn—Al ternary alloys.

The following Table V shows the effect on mechanical properties of additions of other alpha promoters, as well as beta promoters and compound formers to the Ti—Sb base alloys of the invention. With respect to additions of beta promoters of the beta isomorphous group, additions of up to 15% molybdenum are shown to result in a tremendous enhancement in tensile strength while retaining the alloy in extremely ductile condition. For the Ti—4% Sb base alloy, the tensile strength is approximately doubled by additions of up to 12% molybdenum while maintaining the minimum bend ductility under 2.8T. Similar results are obtained for corresponding additions to the Ti—(8–12%) Sb base alloys. These same remarks are likewise applicable to additions of the remaining elements of the beta isomorphous group to the base

5  
10  
15  
20  
25

alloy i. e., vanadium, columbium and tantalum. In each instance there is a marked enhancement in strength with practically no loss in ductility. With respect to the eutectoid beta promoters, those which are sluggishly reactive, such as iron, manganese and chromium, greatly strengthen the alloy without unduly embrittling the same. Thus, for example, the addition of up to 5% iron to the Ti—10% Sb base alloy, increases the ultimate strength from 101,000 to 159,000 p. s. i., while maintaining a minimum bend ductility of not over 4.3T. About the same strengthening effect results from corresponding manganese and chromium additions with no loss in ductility. Thus the addition of up to 4% chromium to the Ti—10% Sb base, increases the ultimate strength from 101,000 to 143,000 p. s. i., while retaining the bend ductility constant at 1.7T. The addition of up to 8% manganese to the Ti—8% Sb base increases the ultimate strength from 88,000 to 157,000 p. s. i., while retaining a bend ductility of not over 2.6T. As regards the rapidly decomposing eutectoid beta promoters and the compound formers such as silicon, boron, arsenic, etc., the strengthening action is not so great, and likewise these elements when present in appreciable amounts, are decidedly more embrittling in their effect.

TABLE V  
*Mechanical properties of Ti—Sb base alloys plus additions of alpha promoters, beta promoters and compound formers (Commercial purity Ti-base)*

[These alloys were 1800° F. forged, 1400° F. rolled to 0.1", descaled, 1300° F. rolled to 0.040", held 15 minutes at 1300° F., furnace cooled to 1100° F., held 1 hour at 1100° F., air cooled to room temperature (stabilizing treatment).]

| Composition, Percent (Balance Titanium) | Tensile Properties: p. s. i. $\times 1000$ |                   |                          | Vickers Hardness | MBR, T |                |
|-----------------------------------------|--------------------------------------------|-------------------|--------------------------|------------------|--------|----------------|
|                                         | 0.2% Offset Yield                          | Ultimate Strength | Percent Elongation in 1" |                  | L      | T              |
| 8Mo                                     | 120                                        | 121               | 10                       | 32               | 248    | 1.5 1.4        |
| 12Mo                                    | 108                                        | 6                 | 37                       | 207              | 1.3    | 2.8            |
| 4Sb                                     | 68                                         | 80                | 20                       | 51               | 180    | 1.6 1.4        |
| 4Sb—8Mo                                 | 118                                        | 120               | 4                        | 22               | 255    | 1.7 2.8        |
| 4Sb—12Mo                                | 121                                        | 122               | 6                        | 30               | 268    | 1.3 2.7        |
| 8Sb                                     | 78                                         | 88                | 20                       | 53               | 206    | 1.8 1.8        |
| 8Sb—2Mo                                 | 110                                        | 118               | 19                       | 47               | 272    | 1.8 2.7        |
| 8Sb—4Mo                                 | 109                                        | 118               | 13                       | 43               | 263    | 1.7 1.8        |
| 8Sb—6Mo                                 | 118                                        | 125               | 9                        | 32               | 273    | 1.8 1.8        |
| 8Sb—8Mo                                 | 113                                        | 136               | 7                        | 22               | 305    | 1.5 2.6        |
| 8Sb—12Mo                                | 128                                        | 133               | 6                        | 24               | 279    | 0.4 1.8        |
| 10Sb—5Mo                                | 129                                        | 133               | 8                        | 33               | 333    | 1.5 2.3        |
| 10Sb—15Mo                               | 126                                        | 130               | 12                       | 30               | 287    | 0 0            |
| 12Sb                                    | 101                                        | 108               | 19                       | 47               | 235    | 2.7 2.6        |
| 12Sb—2Mo                                | 133                                        | 135               | 9                        | 11               | 292    | 2.4 4.9        |
| 12Sb—4Mo                                | 142                                        | 146               | 7                        | 40               | 299    | 2.7 3.5        |
| 12Sb—8Mo                                | 142                                        | 145               | 7                        | 29               | 299    | 1.3 2.6        |
| 8V                                      | 112                                        | 115               | 11                       | 31               | 272    | 1.2 1.6        |
| 12V                                     | 117                                        | 118               | 5                        | 40               | 281    | 1.5 2.9/5.8    |
| 4Sb                                     | 68                                         | 80                | 20                       | 51               | 180    | 1.6 1.4        |
| 4Sb—8V                                  | 120                                        | 124               | 8                        | 36               | 285    | 1.8 3.0/6.0    |
| 4Sb—12V                                 | 124                                        | 131               | 8                        | 27               | 287    | 2.1 6.8        |
| 8Sb                                     | 78                                         | 88                | 20                       | 53               | 206    | 1.8 1.8        |
| 8Sb—2V                                  | 110                                        | 111               | 18                       | 55               | 317    | 2.3 2.0        |
| 8Sb—4V                                  | 120                                        | 126               | 15                       | 45               | 310    | 1.8 1.9/3.8    |
| 8Sb—6V                                  | 120                                        | 126               | 8                        | 35               | 294    | 0.5 2.1/5.7    |
| 8Sb—8V                                  | 130                                        | 144               | 6                        | 41               | 306    | 2.3 4.5        |
| 8Sb—12V                                 | 130                                        | 144               | 7                        | 33               | 309    | 2.6/7.1 Br     |
| 10Sb—5V                                 | 125                                        | 129               | 11                       | 41               | 323    | 1.6 4.7        |
| 10Sb—15V                                | 125                                        | 131               | 6                        | 26               | 305    | 2.4 5.4        |
| 12Sb                                    | 95                                         | 101               | 17                       | 51               | 227    | 1.7 1.8        |
| 12Sb—2V                                 | 120                                        | 130               | 14                       | 48               | 336    | 2.7 2.7        |
| 12Sb—4V                                 | 133                                        | 138               | 7                        | 41               | 336    | 2.2 1.6        |
| 12Sb—8V                                 | 138                                        | 143               | 6                        | 38               | 333    | 1.8/5.2 5.5/Br |
| 10Sb—10Ta                               | 117                                        | 117               | 17                       | 45               | 327    | 1.5 1.9        |
| 10Sb—10Cb                               | 126                                        | 131               | 10                       | 28               | 318    | 2.0 4.9        |
| 12Cb                                    | 96                                         | 111               | 18                       | 43               | 275    | 1.0 0.9        |
| 16Cb                                    | 107                                        | 117               | 10                       | 39               | 277    | 0.7 1.6        |
| 20Cb                                    | 105                                        | 115               | 8                        | 28               | 290    | 0.9 10.5       |
| 4Sb—8Cb                                 | 93                                         | 110               | 20                       | 50               | 288    | 1.5 1.6        |
| 4Sb—12Cb                                | 94                                         | 119               | 19                       | 45               | 280    | 1.4 1.8        |
| 4Sb—16Cb                                | 97                                         | 123               | 16                       | 35               | 268    | 1.2 6.4        |
| 8Sb—4Cb                                 | 111                                        | 116               | 18                       | 45               | 315    | 2.7 2.8        |
| 8Sb—8Cb                                 | 138                                        | 141               | 7                        | 31               | 321    | 1.1 2.8        |
| 8Sb—12Cb                                | 123                                        | 135               | 12                       | 28               | 293    | 1.8 2.9        |
| 12Sb—4Cb                                | 126                                        | 126               | 12                       | 50               | 338    | 11.3 2.8       |
| 12Sb—8Cb                                | 141                                        | 142               | 12                       | 40               | 342    | 2.4 2.7        |
| 100Ti                                   | 42                                         | 59                | 28                       | 50               | —      | 1.4 1.3        |
| 4Cr                                     | 93                                         | 105               | 15                       | 24               | 270    | 1.6 1.7        |
| 8Cr                                     | 116                                        | 132               | 19                       | 50               | 318    | 1.6 2.4        |
| 4Sb                                     | 68                                         | 80                | 20                       | 51               | —      | 1.6 1.4        |
| 4Sb—4Cr                                 | 106                                        | 123               | 18                       | 39               | 319    | 2.5 5.7        |

TABLE V—Continued

Mechanical properties of Ti—Sb base alloys plus additions of alpha promoters, beta promoters and compound formers (Commercial purity Ti-base)—Con.

| Composition, Percent (Balance Titanium) | Tensile Properties: p. s. i. $\times 1000$ |                   |                          | Percent Reduction in Area | Vickers Hardness | MBR, T |          |
|-----------------------------------------|--------------------------------------------|-------------------|--------------------------|---------------------------|------------------|--------|----------|
|                                         | 0.2% Offset Yield                          | Ultimate Strength | Percent Elongation in 1" |                           |                  | L      | T        |
| 4Sb—8Cr                                 | 123                                        | 142               | 14                       | 26                        | 332              | 2.0    | 2.5      |
| 8Sb                                     | 78                                         | 88                | 20                       | 53                        | 337              | 1.8    | 1.8      |
| 8Sb—4Cr                                 | 116                                        | 134               | 14                       | 23                        | 322              | 2.0    | 2.4      |
| 8Sb—8Cr                                 | 129                                        | 144               | 16                       | 29                        | 338              | 1.0    | 2.4      |
| 10Sb                                    | 95                                         | 101               | 17                       | 51                        | 332              | 1.7    | 1.8      |
| 10Sb—1Cr                                | 124                                        | 125               | 20                       | 46                        | 337              | 2.4    | 2.0      |
| 10Sb—2Cr                                | 126                                        | 131               | 19                       | 31                        | 330              | 2.5    | 2.5      |
| 10Sb—4Cr                                | 131                                        | 143               | 9                        | 5                         | 343              | 1.7    | 1.5      |
| 10Sb—5Cr                                | 140                                        | 144               | 11                       | 26                        | 316              | 5.1    |          |
| 12Sb                                    | 101                                        | 108               | 19                       | 47                        | 337              | 2.7    | 2.6      |
| 12Sb—1Cr                                | 123                                        | 124               | 16                       | 44                        | 353              | 1.5    | 3.5      |
| 12Sb—2Cr                                | 142                                        | 148               | 15                       | 47                        | 345              | 3.7    | 2.5      |
| 12Sb—3Cr                                | 135                                        | 144               | 15                       | 30                        | 354              | 2.5    | 2.5      |
| 12Sb—4Cr                                | 135                                        | 147               | 13                       | 17                        | 358              | 1.7    | 2.4      |
| 14Sb                                    | 114                                        | 116               | 12                       | 48                        | 337              | 2.5    | 2.6      |
| 14Sb—1Cr                                | 142                                        | 142               | 15                       | 35                        | 350              | 9.4    | 4.7      |
| 14Sb—2Cr                                | 139                                        | 153               | 12                       | 26                        | 358              | 2.3    | 2.3      |
| 4Mn                                     | 93                                         | 112               | 20                       | 40                        | 273              | 1.3    | 1.4      |
| 6Mn                                     | 113                                        | 126               | 19                       | 42                        | 322              | 2.0    | 1.5      |
| 8Mn                                     | 112                                        | 133               | 20                       | 32                        | 337              | 1.1    | 2.1      |
| 2Sb                                     | 70                                         | 88                | 20                       | 47                        | 191              | 1.8    | 0.9      |
| 2Sb—4Mn                                 | 100                                        | 116               | 20                       | 45                        | 301              | 1.3    | 1.3      |
| 2Sb—6Mn                                 | 118                                        | 132               | 20                       | 31                        | 318              | 1.1    | 1.5      |
| 2Sb—8Mn                                 | 123                                        | 142               | 13                       | 28                        | 347              | 0.8    | 2.5/10.0 |
| 4Sb                                     | 68                                         | 80                | 20                       | 51                        | 180              | 1.6    | 1.4      |
| 4Sb—2Mn                                 | 90                                         | 104               | 13                       | 31                        | 298              | 1.8    | 1.1      |
| 4Sb—4Mn                                 | 111                                        | 127               | 12                       | 26                        | 329              | 1.1    | 1.7      |
| 4Sb—6Mn                                 | 118                                        | 137               | 13                       | 30                        | 330              | 1.5    | 2.0      |
| 4Sb—8Mn                                 | 126                                        | 142               | 13                       | 31                        | 345              | 0.8    | 3.8      |
| 6Sb                                     | 74                                         | 85                | 21                       | 57                        | 192              | 1.6    | 1.4      |
| 6Sb—2Mn                                 | 104                                        | 116               | 15                       | 41                        | 321              | 1.6    | 1.5      |
| 6Sb—4Mn                                 | 118                                        | 132               | 15                       | 33                        | 328              | 1.5    | 2.1      |
| 6Sb—6Mn                                 | 132                                        | 146               | 8                        | 22                        | 356              | 1.3    | 2.2      |
| 6Sb—8Mn                                 | 139                                        | 153               | 12                       | 23                        | 358              | 1.2    | 2.7      |
| 8Sb                                     | 78                                         | 88                | 20                       | 53                        | 206              | 1.8    | 1.8      |
| 8Sb—1Mn                                 | 104                                        | 110               | 18                       | 43                        | 325              | 2.8    | 1.8      |
| 8Sb—2Mn                                 | 108                                        | 115               | 18                       | 43                        | 334              | 2.8    | 2.7      |
| 8Sb—3Mn                                 | 115                                        | 125               | 15                       | 29                        | 330              | 2.7    | 2.3      |
| 8Sb—4Mn                                 | 129                                        | 137               | 10                       | 30                        | 345              | 1.7    | 1.7      |
| 8Sb—6Mn                                 | 138                                        | 148               | 11                       | 27                        | 362              | 1.5    | 2.6      |
| 8Sb—8Mn                                 | 146                                        | 157               | 10                       | 25                        | 360              | 1.2    | 2.6      |
| 10Sb                                    | 95                                         | 101               | 17                       | 51                        | 227              | 1.7    | 1.8      |
| 10Sb—2Mn                                | 119                                        | 123               | 16                       | 44                        | 342              | 2.6    | 1.8      |
| 10Sb—3Mn                                | 130                                        | 133               | 12                       | 43                        | 328              | 1.5    |          |
| 10Sb—4Mn                                | 139                                        | 150               | 15                       | 20                        | 362              | 1.7    | 2.6      |
| 10Sb—6Mn                                | 140                                        | 153               | 13                       | 30                        | 372              | 1.4    | 3.8      |
| 12Sb                                    | 101                                        | 108               | 19                       | 47                        | 235              | 2.7    | 2.6      |
| 12Sb—1Mn                                | 121                                        | 128               | 16                       | 39                        | 336              | 2.7    | 2.7      |
| 12Sb—2Mn                                | 119                                        | 126               | 19                       | 36                        | 352              | 3.1    | 2.5      |
| 12Sb—3Mn                                | 141                                        | 150               | 15                       | 37                        | 350              | 1.7    | 2.2      |
| 12Sb—4Mn                                | 144                                        | 153               | 13                       | 29                        | 354              | 1.9    | 2.6      |
| 14Sb                                    | 114                                        | 116               | 12                       | 48                        | 238              | 2.5    | 2.6      |
| 14Sb—1Mn                                | 134                                        | 135               | 15                       | 26                        | 356              | 2.9    | 2.5      |
| 14Sb—2Mn                                | 144                                        | 148               | 14                       | 27                        | 372              | 5.1    | 2.6      |
| 2Fe                                     | 71                                         | 98                | 18                       | 45                        | 249              | 1.5    | 2.2      |
| 2Sb                                     | 70                                         | 88                | 20                       | 47                        | 191              | 1.3    | 0.9      |
| 2Sb—6Fe                                 | 132                                        | 134               | 0                        | 5                         | 356              | 10.0   | 10.1     |
| 4Sb                                     | 68                                         | 80                | 20                       | 51                        | 180              | 1.6    | 1.4      |
| 4Sb—4Fe                                 | 113                                        | 136               | 8                        | 16                        | 338              | 9.3    | 11.0     |
| 6Sb                                     | 74                                         | 85                | 21                       | 57                        | 192              | 1.6    | 1.4      |
| 6Sb—2Fe                                 | 91                                         | 102               | 20                       | 44                        | 300              | 2.8    | 2.3      |
| 6Sb—6Fe                                 | 139                                        | 157               | 9                        | 19                        | 372              | 8.4    | 7.5      |
| 8Sb                                     | 78                                         | 88                | 20                       | 53                        | 206              | 1.8    | 1.8      |
| 8Sb—2Fe                                 | 114                                        | 126               | 18                       | 37                        | 333              | 4.1    | 1.8      |
| 8Sb—4Fe                                 | 131                                        | 144               | 4                        | 8                         | 361              | 6.1    | 4.0      |
| 10Sb                                    | 95                                         | 101               | 17                       | 51                        | 227              | 1.7    | 1.8      |
| 10Sb—1Fe                                | 115                                        | 121               | 15                       | 39                        | 337              | 2.8    | 2.7      |
| 10Sb—2Fe                                | 118                                        | 123               | 12                       | 21                        | 348              | 7.7    | 4.2      |
| 10Sb—2.5Fe                              | 132                                        | 139               | 11                       | 34                        | 337              | 2.3    |          |
| 10Sb—5Fe                                | 143                                        | 159               | 4                        | 3                         | 360              | 1.0    | 4.3      |
| 10Sb—6Fe                                | 157                                        | 165               | 3                        | 6                         | 393              | 10.1   | 9.8      |
| 12Sb                                    | 101                                        | 108               | 19                       | 47                        | 235              | 2.7    | 2.6      |
| 12Sb—1Fe                                | 121                                        | 126               | 10                       | 26                        | 355              | 5.0    | 4.2      |
| 12Sb—2Fe                                | 133                                        | 142               | 7                        | 15                        | 361              | 6.4    | 5.5      |
| 12Sb—4Fe                                | 154                                        | 163               | 3                        | 5                         | 389              | 10.4   | 10.4     |
| 14Sb                                    | 114                                        | 116               | 12                       | 48                        | 238              | 2.5    | 2.6      |
| 14Sb—1Fe                                | 133                                        | 138               | 8                        | 18                        | 383              | 5.3    | 4.4      |
| 14Sb—2Fe                                | 148                                        | 154               | 5                        | 13                        | 375              | 7.6    | 7.9      |
| 10Sb—5W                                 | 96                                         | 107               | 20                       | 39                        | 318              | 2.3    | 2.3      |
| 10Sb—2.5Cu                              | 129                                        | 136               | 8                        | 20                        | 344              | 2.3    |          |
| 10Sb—2.5Co                              | 108                                        | 119               | 11                       | 28                        | 309              | 5.4    |          |
| 10Sb—2.5Ni                              | 97                                         | 109               | 17                       | 56                        | 296              | 2.5    | 5.7      |
| 10Sb—1Si                                | 97                                         | 108               | 15                       | 34                        | 317              | 2.3    | 4.7      |
| 10Sb—2.5O                               | 86                                         | 95                | 9                        | 17                        | 281              | 5.5    |          |
| 10Sb—0.5B                               | 79                                         | 95                | 18                       | 35                        | 280              | 2.7    | 7.1      |
| 10Sb—0.5As                              | 92                                         | 102               | 18                       | 33                        | 305              | 2.7    | 5.2      |
| 10Sb—0.5S                               | 96                                         | 105               | 4                        | 10                        | 317              | 2.8    | 5.5      |
| 10Sb—0.5Te                              | 85                                         | 97                | 18                       | 43                        | 292              | 1.7    | 3.5      |
| 10Sb—0.5P                               | 98                                         | 108               | 20                       | 39                        | 315              | 2.7    |          |
| 10Sb—10Ag                               | 101                                        | 115               | 17                       | 40                        | 318              | 2.7    | 5.3      |
| 10Sb—10In                               | 111                                        | 120               | 12                       | 37                        | 330              | 2.3    | 4.6      |
| 10Sb—5Bi (added)                        | 92                                         | 103               | 19                       | 34                        | 309              | 2.7    | 3.5      |
| 10Sb—10Pb (added)                       | 95                                         | 107               | 16                       | 42                        | 305              | 1.7    | 3.4      |
| 10Sb—2.5Ti                              | 83                                         | 94                | 17                       | 45                        | 291              | 1.7    | 3.3      |

TABLE V—Continued

Mechanical properties of Ti—Sb base alloys plus additions of alpha promoters, beta promoters and compound formers (Commercial purity Ti-base)—Con.

[The following alloys were 1,800° F. forged, 1,400° F. rolled to 0.1", descaled, 1,400° F. rolled to 0.04", annealed 15 minutes at 1,400° F. or at 1,550° F., the latter as indicated by an asterisk, and quenched (beta fabrication treatment).]

| Composition, Percent (Balance Titanium) | Tensile Properties: p. s. i. $\times 1000$ |                   |                          | Vickers Hardness | MBR, T |         |
|-----------------------------------------|--------------------------------------------|-------------------|--------------------------|------------------|--------|---------|
|                                         | 0.2% Offset Yield                          | Ultimate Strength | Percent Elongation in 1" |                  | L      | T       |
| 12Mo                                    | 125                                        | 126               | 6                        | 36               | 343    | 1.0     |
| 45B—12Mo                                | 69                                         | 110               | 8                        | 26               | 251    | 1.0     |
| 85B—12Mo                                | 115                                        | 130               | 5                        | 35               | 287    | 0       |
| 16Mo                                    | 110                                        | 123               | 10                       | 37               | 276    | 0       |
| 45B—16Mo                                | 117                                        | 122               | 7                        | 39               | 260    | 0       |
| 85B—16Mo                                | 119                                        | 123               | 8                        | 38               | 268    | 0       |
| 20Mo                                    | 120                                        | 121               | 6                        | 33               | 266    | 0       |
| 40Mo                                    | 116                                        | 118               | 1                        | 0                | 312    | 0/1.9   |
| 45B—40Mo                                | (1)                                        | (1)               | (1)                      | (1)              | (1)    | (1)     |
| 12V                                     |                                            | 120               | 1                        | 0                | V Br   | V Br    |
| 45B—12V                                 | 131                                        | 142               | 1                        | 3                | 312    | 5.8/Br  |
| 85B—12V                                 | 129                                        | 138               | 5                        | 28               | 314    | 2.8/Br  |
| 16V                                     | 164                                        | 166               | 1                        | 0                | 386    | V Br    |
| 45B—16V                                 | 140                                        | 144               | 5                        | 29               | 317    | 1.9     |
| 85B—16V                                 | 137                                        | 144               | 4                        | 27               | 306    | 1.9/5.7 |
| 20V                                     | 145                                        | 138               | 6                        | 24               | 326    | 2.5/4.9 |
| 40V                                     | 150                                        | 150               | 1                        | 2                | 350    | 5.7/Br  |
| 45B—40V                                 | (1)                                        | (1)               | (1)                      | (1)              | (1)    | (1)     |
| 0.55B—30Mo*                             | 133                                        | 133               | 8                        | 33               | 296    | 0.9     |
| 0.55B—30V*                              | 103                                        | 108               | 12                       | 30               | 236    | 0       |
| 0.55B—40V*                              | 111                                        | 115               | 10                       | 33               | 256    | 0       |
| 0.55B—30Cb*                             | 68                                         | 85                | 14                       | 28               | 203    | 0.5     |
| 0.55B—30Ta*                             | 69                                         | 100               | 14                       | 28               | 209    | 0.5     |
| 0.55B—30Zr*                             | 109                                        | 142               | 5                        | 6                | 308    | 6.0     |
| 8Cr                                     | 189                                        | 190               | 3                        | 10               | 423    | 3.5     |
| 12Cr                                    | 140                                        | 145               | 10                       | 27               | 336    | 0       |
| 16Cr                                    | 141                                        | 150               | 10                       | 26               | 336    | 0       |
| 20Cr                                    | 139                                        | 155               | 6                        | 11               | 387    | 0.9     |
| 25B—20Cr                                | 149                                        | 157               | 5                        | 10               | 350    | 1.8     |
| 45B—8Cr                                 | 136                                        | 150               | 6                        | 24               | 346    | 0.9     |
| 45B—12Cr                                | 135                                        | 144               | 14                       | 31               | 335    | 1.2     |
| 45B—16Cr                                | 147                                        | 154               | 3                        | 6                | 360    | 4.2     |
| 85B—8Cr                                 | 137                                        | 144               | 8                        | 33               | 323    | 0.4     |
| 85B—12Cr                                | 142                                        | 143               | 9                        | 32               | 328    | 0.4     |

\* Could not be fabricated.

Referring to the above table, it will be seen that the Ti—Sb—(Mo, V, Cb, Ta) alloys when given the stabilizing treatment, have very similar properties. On the other hand, when these alloys are given the beta fabrication treatment, the Ti—Sb—V alloys are shown to have higher strengths and much lower ductilities than the corresponding Ti—Sb—Mo alloys.

The following Table VI gives elevated temperature test results on oxidation and contamination resistance of alloys according to the invention:

TABLE VI  
Oxidation data for Ti—Sb alloys

[Heated 4 hours at 1050° C. in air and furnace cooled.]

| Composition, Percent, (Balance Titanium) | Weight Gain, g./dm. <sup>2</sup> | Metal Thickness Loss, mils | Depth of Contamination, mils | Increase in VHN, 5 mils below surface |
|------------------------------------------|----------------------------------|----------------------------|------------------------------|---------------------------------------|
| 100Ti                                    | 3.45                             | 10                         | 60                           | 210                                   |
| 5Sb                                      | 4.72                             | 5                          | 60                           | 200                                   |
| 10Sb                                     | 4.35                             | 4                          | 40                           | 110                                   |
| 15Sb                                     | 7.00                             | 7                          | Nil                          | Nil                                   |

From the above it will be seen that these alloys are quite resistant to oxidation and to penetration by atmospheric gases at temperatures as high as 1050° C.

The following Table VII gives data on the welding characteristics of alloys in accordance with the invention as arc welded in an inert atmosphere, in this case, argon.

45

TABLE VII  
Bend ductility of welded Ti—Sb, Ti—Sb—Sn and Ti—Sb—Al alloys  
(IODIDE Ti BASE)

| Composition, Percent (Balance Titanium) | Minimum Bend Radius, T |            |
|-----------------------------------------|------------------------|------------|
|                                         | Welded                 | Not Welded |
| 100Ti                                   | 1.0                    | 0          |
| 2.6Sb                                   | 0                      | 0          |
| 5Sb                                     | 1.1                    | 0.6        |
| 7.5Sb                                   | 0.6                    | 1.6        |
| 10Sb                                    |                        | 1.9        |
| 12.5Sb                                  |                        | 2.4        |
| 15Sb                                    | 2.2                    | 3.4        |
| 17.5Sb                                  | 3.4                    | 3.7        |
| COMMERCIAL PURITY Ti BASE               |                        |            |
| 100Ti                                   | 1.5                    | 0.8        |
| 1Sb                                     | 2.3                    | 0.4        |
| 2.6Sb                                   | 1.5                    | 1.2        |
| 5Sb                                     | 2.4                    | 1.5        |
| 10Sb                                    | 4.4                    | 1.5        |
| 14Sb                                    | 2.6                    | 2.3        |
| 16Sb                                    | 4.9                    | 2.5        |
| 17Sb                                    | 5.0                    | 2.5        |
| 18Sb                                    | Br                     | 4.8        |
| 18Sb                                    | 7.3                    | Br         |
| 18Sb                                    | Br                     | 4.8        |
| 5Sb                                     | 2.4                    | 1.5        |
| 5Sb—5Sn                                 | 4.7                    | 1.5        |
| 5Sb—10Sn                                | 6.6                    | 1.7        |
| 5Sb—15Sn                                |                        | 2.0        |
| 5Sb—17.5Sn                              |                        | 2.0        |
| 10Sb                                    | 4.4                    | 1.5        |
| 10Sb—5Sn                                | 4.3                    | 2.5        |
| 10Sb—10Sn                               | Br                     | 4.9        |
| 10Sb—12.5Sn                             | V Br                   | Br         |

TABLE VII—Continued

Bend ductility of welded Ti—Sb, Ti—Sb—Sn and  
Ti—Sb—Al alloys—Continued  
(COMMERCIAL PURITY Ti BASE)—Continued

| Composition, Percent (Balance Titanium) | Minimum Bend Radius, T |            | 10 | Composition, Percent (Balance Titanium) | Minimum Bend Radius, T |            |
|-----------------------------------------|------------------------|------------|----|-----------------------------------------|------------------------|------------|
|                                         | Welded                 | Not Welded |    |                                         | Welded                 | Not Welded |
| 10Sb                                    | 4.4                    | 1.5        |    | 4Mn                                     | Br                     | 1.3        |
| 7.5Sb—2.5Sn                             |                        | 2.1        |    | 6Mn                                     | Br                     | 2.0        |
| 5Sb—5Sn                                 | 4.7                    | 1.5        |    | 8Mn                                     | Br                     | 1.1        |
| 2.5Sb—7.5Sn                             | 1.1                    | 2.2        |    | 2Sb—4Mn                                 | Br                     | 1.3        |
| 10Sn                                    | 3.2                    | 1.7        | 15 | 2Sb—6Mn                                 | Br                     | 1.1        |
| 15Sb                                    | 4.9                    | 2.5        |    | 2Sb—8Mn                                 | Br                     | 0.8        |
| 12.5Sb—2.5Sn                            | 7.6                    | 1.9        |    | 4Sb—2Mn                                 | 5.7                    | 1.8        |
| 10Sb—8Sn                                | 4.3                    | 2.5        |    | 4Sb—4Mn                                 | Br                     | 1.1        |
| 6Sb—10Sn                                | 6.6                    | 1.7        |    | 4Sb—6Mn                                 | Br                     | 1.5        |
| 2.5Sb—12.5Sn                            | 5.7                    | 2.9        |    | 4Sb—8Mn                                 | Br                     | 0.8        |
| 15Sn                                    | 3.4                    | 1.8        |    | 6Sb—2Mn                                 | Br                     | 1.6        |
| 5Sb                                     | 2.4                    | 1.5        | 20 | 6Sb—4Mn                                 | Br                     | 1.5        |
| 5Sb—1Al                                 | 1.5                    | 2.1        |    | 6Sb—6Mn                                 | Br                     | 1.3        |
| 5Sb—2Al                                 | 4.2                    | 1.5        |    | 6Sb—8Mn                                 | Br                     | 1.2        |
| 5Sb—3Al                                 | 1.9                    | 2.1        |    | 8Sb—1Mn                                 | Br                     | 2.8        |
| 5Sb—4Al                                 | 5.2                    | 2.7        |    | 8Sb—2Mn                                 | 11.6                   | 2.8        |
| 10Sb                                    | 4.4                    | 1.5        |    | 8Sb—3Mn                                 | Br                     | 2.7        |
| 10Sb—1Al                                | 1.9                    | 2.1        | 25 | 8Sb—4Mn                                 | Br                     | 2.7        |
| 10Sb—2Al                                | 5.2                    | 2.5        |    | 8Sb—6Mn                                 | Br                     | 1.5        |
| 10Sb—3Al                                | 2.9                    | 2.8        |    | 8Sb—8Mn                                 | Br                     | 1.2        |
| 10Sb—4Al                                | Br                     | 2.5        |    | 10Sb—2Mn                                | Br                     | 2.6        |
| 10Sb—5Al                                | V Br                   |            |    | 10Sb—4Mn                                | 10.6                   | 1.7        |
| 12.5Sb                                  | 5.8                    | 2.6        |    | 10Sb—6Mn                                | Br                     | 1.4        |
| 12.5Sb—1Al                              | 5.8                    | 2.1        |    | 12Sb—1Mn                                | 7.1                    | 2.7        |
| 12.5Sb—2Al                              | 2.9                    | 2.3        |    | 12Sb—2Mn                                | Br                     | 3.1        |
| 12.5Sb—3Al                              | >7                     | Br         |    | 12Sb—3Mn                                | Br                     | 1.7        |
| 15Sb                                    | 4.9                    | 2.5        | 30 | 12Sb—4Mn                                | 5.3                    | 1.9        |
| 15Sb—1Al                                | 7.6                    | 3.1        |    | 14Sb—1Mn                                | 11.0                   | 2.9        |
| 15Sb—2Al                                | V Br                   | Br         |    | 14Sb—2Mn                                | Br                     | 5.9        |
| 15Sb—3Al                                | V Br                   | Br         |    | 4Cr                                     | Br                     | 1.6        |
| 17Sb                                    | 7.3                    | Br         |    | 8Or                                     | Br                     | 1.6        |
| V Br                                    | Br                     |            |    | 4Sb—4Cr                                 | Br                     | 2.5        |
| 17.5Sb—1Al                              | 5.7                    | 2.8        |    | 4Sb—8Cr                                 | Br                     | 2.0        |
| 7.5Sb—4Al                               |                        |            |    | 8Sb—8Cr                                 | 1.5                    | 1.0        |
| 10Sb—2.5Al                              | 5.0                    | 2.4        | 35 | 10Sb—1Cr                                | 6.8                    | 2.4        |
| 7.5Sb—2.5Sn—2.5Al                       | 4.9                    | 2.6        |    | 10Sb—2Cr                                | Br                     | 2.5        |
| 6Sb—5Sn—2.5Al                           | 2.6                    | 2.8        |    | 10Sb—4Cr                                | 10.6                   | 1.7        |
| 2.5Sb—7.5Sn—2.5Al                       | >7                     | 2.6        |    | 12Sb—1Cr                                | 9.6                    | 1.5        |
| 10Sn—2.5Al                              | >8                     | 2.5        |    | 12Sb—2Cr                                | 6.6                    | 3.7        |
| V Br                                    | 2.0                    |            |    | 12Sb—3Cr                                | Br                     | 2.5        |
| 6.4                                     | 2.5                    |            |    | 12Sb—4Cr                                | 10.4                   | 1.7        |
| V Br                                    | 6.2                    |            |    | 14Sb—1Cr                                | Br                     | 9.4        |
| V Br                                    | 3.0                    |            | 40 | 14Sb—2Cr                                | 7.0                    | 2.3        |
| V Br                                    | 5.5                    |            |    | 0.55Sb—30Mo                             | Br                     | 0.9        |
| 2.8                                     | 2.8                    |            |    | 0.55Sb—30V                              | 1.8                    | 0          |
| 5Al—2.5Sb                               | 5.7                    | 2.8        |    | 0.55Sb—40V                              | 7.1                    | 0          |
| 5Al—2Sb—0.5Sn                           |                        |            |    | 0.55Sb—30Ta                             | 0.5                    | 0.5        |
| 5Al—1.5Sb—1Sn                           | 3.1                    | 2.1        |    | 0.55Sb—30Cb                             | 0.5                    | 0.9        |
| 5A—1Sb—1.5Sn                            | 2.9                    | 2.9        |    | 0.55Sb—30Zr                             | Br                     | 6.0        |
| 5Al—0.5Sb—2Sn                           | 2.8                    |            |    |                                         |                        |            |
| 5Al—2.5Sn                               | 3.8                    |            |    |                                         |                        |            |
| 5Al—2.5Sb—0.2C                          | 5.5                    |            |    |                                         |                        |            |
| 5Al—1.5Sb—1.5Sn—0.2C                    | 5.2                    |            |    |                                         |                        |            |
| 5Al—1Sb—1.5Sn—0.2C                      | 7.3                    |            |    |                                         |                        |            |
| 5Al—0.5Sb—2Sn—0.2C                      | >7                     |            |    |                                         |                        |            |
| 5Al—2.5Sb—0.2C                          | V Br                   | 2.8        |    |                                         |                        |            |
| 4Sb—8Mo                                 | 1.9                    | 1.7        |    |                                         |                        |            |
| 4Sb—12Mo                                | 0                      | 1.3        |    |                                         |                        |            |
| 8Sb—2Mo                                 | 3.0                    | 1.8        |    |                                         |                        |            |
| 8Sb—4Mo                                 | 2.0                    | 1.8        |    |                                         |                        |            |
| 8Sb—6Mo                                 | 1.9                    | 1.8        |    |                                         |                        |            |
| 8Sb—8Mo                                 | 1.5                    | 1.5        |    |                                         |                        |            |
| 8Sb—12Mo                                | 0                      | 0.4        |    |                                         |                        |            |
| 12Sb—2Mo                                | 2.6                    | 2.4        |    |                                         |                        |            |
| 12Sb—4Mo                                | 3.6                    | 2.7        |    |                                         |                        |            |
| 12Sb—8Mo                                | 2.8                    | 1.3        |    |                                         |                        |            |
| 12Mo                                    | 1.5                    | 1.0        |    |                                         |                        |            |
| 16Mo                                    | 0                      | 0          |    |                                         |                        |            |
| 20Mo                                    | 0                      | 0          |    |                                         |                        |            |
| 40Mo                                    | Br                     | 0/1.9      |    |                                         |                        |            |
| 4Sb—12Mo                                | 1.6                    | 1.0        |    |                                         |                        |            |
| 4Sb—16Mo                                | 1.0                    | 0          |    |                                         |                        |            |
| 8Sb—12Mo                                | 1.1                    | 0          |    |                                         |                        |            |
| 8Sb—16Mo                                | 0.5                    | 0          |    |                                         |                        |            |
| 8Cr                                     | Br                     | 3.5        |    |                                         |                        |            |
| 12Cr                                    | 10.4                   | 0          |    |                                         |                        |            |
| 16Cr                                    | 5.3                    | 0          |    |                                         |                        |            |
| 20Cr                                    | 7.1                    | 0.9        |    |                                         |                        |            |
| 28Sb—20Cr                               | Br                     | 1.8        |    |                                         |                        |            |
| 4Sb—8Cr                                 | Br                     | 0.9        |    |                                         |                        |            |
| 4Sb—12Cr                                | Br                     | 1.2        |    |                                         |                        |            |
| 4Sb—16Cr                                | Br                     | 4.2        |    |                                         |                        |            |
| 8Sb—8Cr                                 | 0.9                    | 0.4        |    |                                         |                        |            |
| 8Sb—12Cr                                | 0.4                    | 0.4        |    |                                         |                        |            |
| 2Sb—6Fe                                 | Br                     | 10.0       |    |                                         |                        |            |
| 4Sb—4Fe                                 | Br                     | 9.3        |    |                                         |                        |            |
| 6Sb—2Fe                                 | 3.7                    | 2.8        |    |                                         |                        |            |
| 6Sb—6Fe                                 | Br                     | 8.4        |    |                                         |                        |            |
| 8Sb—2Fe                                 | Br                     | 4.1        |    |                                         |                        |            |
| 8Sb—4Fe                                 | Br                     | 6.1        |    |                                         |                        |            |
| 10Sb—1Fe                                | Br                     | 2.8        |    |                                         |                        |            |
| 10Sb—2Fe                                | Br                     | 7.7        |    |                                         |                        |            |
| 10Sb—6Fe                                | Br                     | 10.1       |    |                                         |                        |            |
| 12Sb—1Fe                                | Br                     | 5.0        |    |                                         |                        |            |
| 12Sb—2Fe                                | Br                     | 6.4        |    |                                         |                        |            |
| 12Sb—4Fe                                | Br                     | 10.4       |    |                                         |                        |            |
| 14Sb—1Fe                                | Br                     | 5.3        |    |                                         |                        |            |
| 14Sb—2Fe                                | Br                     | 7.6        |    |                                         |                        |            |

TABLE VII—Continued

Bend ductility of welded Ti—Sb, Ti—Sb—Sn and  
Ti—Sb—Al alloys—Continued  
(COMMERCIAL PURITY Ti BASE)—Continued

| Composition, Percent (Balance Titanium)                                                                                                                                                                                                                                                                                                                                                                                                                                                                                                                                                                                                                                                              | Minimum Bend Radius, T |            | 5 | Composition, Percent (Balance Titanium) | Minimum Bend Radius, T |            |
|------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------------|------------------------|------------|---|-----------------------------------------|------------------------|------------|
|                                                                                                                                                                                                                                                                                                                                                                                                                                                                                                                                                                                                                                                                                                      | Welded                 | Not Welded |   |                                         | Welded                 | Not Welded |
| 4Mn                                                                                                                                                                                                                                                                                                                                                                                                                                                                                                                                                                                                                                                                                                  | Br                     | 1.3        |   | 6Mn                                     | Br                     | 2.0        |
| 8Mn                                                                                                                                                                                                                                                                                                                                                                                                                                                                                                                                                                                                                                                                                                  | Br                     | 1.1        |   | 8Mn                                     | Br                     | 1.3        |
| 2Sb—4Mn                                                                                                                                                                                                                                                                                                                                                                                                                                                                                                                                                                                                                                                                                              | Br                     | 1.3        |   | 2Sb—6Mn                                 | Br                     | 1.1        |
| 2Sb—8Mn                                                                                                                                                                                                                                                                                                                                                                                                                                                                                                                                                                                                                                                                                              | Br                     | 0.8        |   | 4Sb—2Mn                                 | 5.7                    | 1.8        |
| 4Sb—4Mn                                                                                                                                                                                                                                                                                                                                                                                                                                                                                                                                                                                                                                                                                              | Br                     | 1.1        |   | 4Sb—4Mn                                 | Br                     | 1.1        |
| 4Sb—6Mn                                                                                                                                                                                                                                                                                                                                                                                                                                                                                                                                                                                                                                                                                              | Br                     | 1.5        |   | 4Sb—8Mn                                 | Br                     | 0.8        |
| 4Sb—8Mn                                                                                                                                                                                                                                                                                                                                                                                                                                                                                                                                                                                                                                                                                              | Br                     | 0.8        |   | 6Sb—2Mn                                 | Br                     | 1.6        |
| 6Sb—2Mn                                                                                                                                                                                                                                                                                                                                                                                                                                                                                                                                                                                                                                                                                              | Br                     | 1.6        |   | 6Sb—4Mn                                 | Br                     | 1.5        |
| 6Sb—4Mn                                                                                                                                                                                                                                                                                                                                                                                                                                                                                                                                                                                                                                                                                              | Br                     | 1.5        |   | 6Sb—6Mn                                 | Br                     | 1.4        |
| 6Sb—6Mn                                                                                                                                                                                                                                                                                                                                                                                                                                                                                                                                                                                                                                                                                              | Br                     | 1.4        |   | 6Sb—8Mn                                 | Br                     | 1.3        |
| 6Sb—8Mn                                                                                                                                                                                                                                                                                                                                                                                                                                                                                                                                                                                                                                                                                              | Br                     | 1.3        |   | 8Sb—1Mn                                 | Br                     | 1.2        |
| 8Sb—1Mn                                                                                                                                                                                                                                                                                                                                                                                                                                                                                                                                                                                                                                                                                              | Br                     | 2.8        |   | 8Sb—2Mn                                 | Br                     | 2.8        |
| 8Sb—2Mn                                                                                                                                                                                                                                                                                                                                                                                                                                                                                                                                                                                                                                                                                              | 11.6                   | 2.8        |   | 8Sb—3Mn                                 | Br                     | 2.7        |
| 8Sb—3Mn                                                                                                                                                                                                                                                                                                                                                                                                                                                                                                                                                                                                                                                                                              | Br                     | 2.7        |   | 8Sb—4Mn                                 | Br                     | 2.7        |
| 8Sb—4Mn                                                                                                                                                                                                                                                                                                                                                                                                                                                                                                                                                                                                                                                                                              | Br                     | 2.7        |   | 8Sb—6Mn                                 | Br                     | 2.6        |
| 8Sb—6Mn                                                                                                                                                                                                                                                                                                                                                                                                                                                                                                                                                                                                                                                                                              | Br                     | 2.6        |   | 8Sb—8Mn                                 | Br                     | 2.6        |
| 8Sb—8Mn                                                                                                                                                                                                                                                                                                                                                                                                                                                                                                                                                                                                                                                                                              | Br                     | 2.6        |   | 10Sb—2Mn                                | Br                     | 2.6        |
| 10Sb—2Mn                                                                                                                                                                                                                                                                                                                                                                                                                                                                                                                                                                                                                                                                                             | Br                     | 2.6        |   | 10Sb—4Mn                                | 10.6                   | 1.7        |
| 10Sb—4Mn                                                                                                                                                                                                                                                                                                                                                                                                                                                                                                                                                                                                                                                                                             | Br                     | 1.7        |   | 10Sb—6Mn                                | Br                     | 1.4        |
| 10Sb—6Mn                                                                                                                                                                                                                                                                                                                                                                                                                                                                                                                                                                                                                                                                                             | Br                     | 1.4        |   | 12Sb—1Mn                                | 7.1                    | 2.7        |
| 12Sb—1Mn                                                                                                                                                                                                                                                                                                                                                                                                                                                                                                                                                                                                                                                                                             | Br                     | 3.1        |   | 12Sb—2Mn                                | Br                     | 3.1        |
| 12Sb—2Mn                                                                                                                                                                                                                                                                                                                                                                                                                                                                                                                                                                                                                                                                                             | Br                     | 3.1        |   | 12Sb—3Mn                                | Br                     | 1.7        |
| 12Sb—3Mn                                                                                                                                                                                                                                                                                                                                                                                                                                                                                                                                                                                                                                                                                             | Br                     | 1.7        |   | 12Sb—4Mn                                | 5.3                    | 1.9        |
| 12Sb—4Mn                                                                                                                                                                                                                                                                                                                                                                                                                                                                                                                                                                                                                                                                                             | Br                     | 1.9        |   | 14Sb—1Mn                                | 11.0                   | 2.9        |
| 14Sb—1Mn                                                                                                                                                                                                                                                                                                                                                                                                                                                                                                                                                                                                                                                                                             | Br                     | 2.9        |   | 14Sb—2Mn                                | Br                     | 5.9        |
| 14Sb—2Mn                                                                                                                                                                                                                                                                                                                                                                                                                                                                                                                                                                                                                                                                                             | Br                     | 5.9        |   | 4Cr                                     | Br                     | 1.6        |
| 4Cr                                                                                                                                                                                                                                                                                                                                                                                                                                                                                                                                                                                                                                                                                                  | Br                     | 1.6        |   | 8Or                                     | Br                     | 1.6        |
| 8Or                                                                                                                                                                                                                                                                                                                                                                                                                                                                                                                                                                                                                                                                                                  | Br                     | 1.6        |   | 4Sb—4Cr                                 | Br                     | 2.5        |
| 4Sb—4Cr                                                                                                                                                                                                                                                                                                                                                                                                                                                                                                                                                                                                                                                                                              | Br                     | 2.5        |   | 4Sb—8Cr                                 | Br                     | 2.0        |
| 4Sb—8Cr                                                                                                                                                                                                                                                                                                                                                                                                                                                                                                                                                                                                                                                                                              | Br                     | 2.0        |   | 8Sb—8Cr                                 | 1.5                    | 1.0        |
| 8Sb—8Cr                                                                                                                                                                                                                                                                                                                                                                                                                                                                                                                                                                                                                                                                                              | Br                     | 1.5        |   | 10Sb—1Cr                                | 6.8                    | 2.4        |
| 10Sb—1Cr                                                                                                                                                                                                                                                                                                                                                                                                                                                                                                                                                                                                                                                                                             | Br                     | 2.4        |   | 10Sb—2Cr                                | Br                     | 2.5        |
| 10Sb—2Cr                                                                                                                                                                                                                                                                                                                                                                                                                                                                                                                                                                                                                                                                                             | Br                     | 2.5        |   | 10Sb—4Cr                                | 10.6                   | 1.7        |
| 10Sb—4Cr                                                                                                                                                                                                                                                                                                                                                                                                                                                                                                                                                                                                                                                                                             | Br                     | 1.7        |   | 12Sb—1Cr                                | 9.6                    | 1.5        |
| 12Sb—1Cr                                                                                                                                                                                                                                                                                                                                                                                                                                                                                                                                                                                                                                                                                             | Br                     | 1.5        |   | 12Sb—2Cr                                | 6.6                    | 3.7        |
| 12Sb—2Cr                                                                                                                                                                                                                                                                                                                                                                                                                                                                                                                                                                                                                                                                                             | Br                     | 2.5        |   | 12Sb—3Cr                                | Br                     | 2.5        |
| 12Sb—3Cr                                                                                                                                                                                                                                                                                                                                                                                                                                                                                                                                                                                                                                                                                             | Br                     | 2.5        |   | 12Sb—4Cr                                | 10.4                   | 1.7        |
| 12Sb—4Cr                                                                                                                                                                                                                                                                                                                                                                                                                                                                                                                                                                                                                                                                                             | Br                     | 1.7        |   | 14Sb—1Cr                                | Br                     | 9.4        |
| 14Sb—1Cr                                                                                                                                                                                                                                                                                                                                                                                                                                                                                                                                                                                                                                                                                             | Br                     | 2.4        |   | 14Sb—2Cr                                | 7.0                    | 2.3        |
| 14Sb—2Cr                                                                                                                                                                                                                                                                                                                                                                                                                                                                                                                                                                                                                                                                                             | Br                     | 2.3        |   | 0.55Sb—30Mo                             | Br                     | 0.9        |
| 0.55Sb—30Mo                                                                                                                                                                                                                                                                                                                                                                                                                                                                                                                                                                                                                                                                                          | Br                     | 0.9        |   | 0.55Sb—30V                              | 1.8                    | 0          |
| 0.55Sb—30V                                                                                                                                                                                                                                                                                                                                                                                                                                                                                                                                                                                                                                                                                           | Br                     | 0          |   | 0.55Sb—40V                              | 7.1                    | 0          |
| 0.55Sb—40V                                                                                                                                                                                                                                                                                                                                                                                                                                                                                                                                                                                                                                                                                           | Br                     | 0          |   | 0.55Sb—30Ta                             | 0.5                    | 0.5        |
| 0.55Sb—30Ta                                                                                                                                                                                                                                                                                                                                                                                                                                                                                                                                                                                                                                                                                          | Br                     | 0          |   | 0.55Sb—30Cb                             | 0.5                    | 0.9        |
| 0.55Sb—30Cb                                                                                                                                                                                                                                                                                                                                                                                                                                                                                                                                                                                                                                                                                          | Br                     | 0          |   | 0.55Sb—30Zr                             | Br                     | 6.0        |
| 0.55Sb—30Zr                                                                                                                                                                                                                                                                                                                                                                                                                                                                                                                                                                                                                                                                                          | Br                     | 0          |   |                                         |                        |            |
| From the above data it will be seen that the alloys of the invention in general suffer no appreciable loss in ductility as a result of welding.                                                                                                                                                                                                                                                                                                                                                                                                                                                                                                                                                      |                        |            |   |                                         |                        |            |
| 50                                                                                                                                                                                                                                                                                                                                                                                                                                                                                                                                                                                                                                                                                                   |                        |            |   |                                         |                        |            |
| The beta-containing alloys of the invention after being given the stabilizing treatment of Table V, are quite stable thermally as shown by aging tests carried out at 400° C. for 48 hours, which are shown to have substantially no effect on the minimum bend ductilities.                                                                                                                                                                                                                                                                                                                                                                                                                         |                        |            |   |                                         |                        |            |
| 55                                                                                                                                                                                                                                                                                                                                                                                                                                                                                                                                                                                                                                                                                                   |                        |            |   |                                         |                        |            |
| The alloys of the invention may be made by melt casting in a cold mold furnace employing an arc electrode in an inert atmosphere, or by other procedures. Where the alloys of the invention are to be used for sheet material, the minimum bend ductility may range as high as 20T, and where used in massive form, as in forgings, the percent tensile elongation may range as low as 1 or 2%.                                                                                                                                                                                                                                                                                                      |                        |            |   |                                         |                        |            |
| What is claimed is:                                                                                                                                                                                                                                                                                                                                                                                                                                                                                                                                                                                                                                                                                  |                        |            |   |                                         |                        |            |
| 1. A titanium base alloy consisting essentially of: about 0.5 to 18% antimony; carbon, oxygen and nitrogen up to 0.6%, 0.4% and 0.3% each, respectively; about 0.5 to 23% of at least one other alpha promoter selected from the group consisting of aluminum, tin, indium, silver, lead and bismuth, but not to exceed 8% of aluminum and 15% in total amount of indium, silver, lead and bismuth; antimony being on the low side of its range when said other alpha promoter content is on the high side of its range and vice versa; the balance of said alloy being substantially titanium, said alloy being characterized by a tensile strength of at least 100,000 p. s. i., a tensile elonga- |                        |            |   |                                         |                        |            |
| 65                                                                                                                                                                                                                                                                                                                                                                                                                                                                                                                                                                                                                                                                                                   |                        |            |   |                                         |                        |            |
| 70                                                                                                                                                                                                                                                                                                                                                                                                                                                                                                                                                                                                                                                                                                   |                        |            |   |                                         |                        |            |
| 75                                                                                                                                                                                                                                                                                                                                                                                                                                                                                                                                                                                                                                                                                                   |                        |            |   |                                         |                        |            |

tion of at least 2% and a minimum bend ductility of at least 20T.

2. A titanium base alloy consisting essentially of: about 0.5 to 18% antimony; carbon, oxygen and nitrogen up to about 0.6%, 0.4% and 0.3% each, respectively; 0.5 to 40% of at least one beta promoter selected from the group consisting of molybdenum, vanadium, columbium, tantalum, zirconium, manganese, iron, chromium, tungsten, cobalt, nickel, copper, silicon and beryllium, but not to exceed about 25% of chromium and tungsten, 10% of manganese, 7% of iron, 5% of cobalt, nickel and copper, and 2% of silicon and beryllium; the balance of said alloy being substantially titanium, and said alloy being characterized by a tensile strength of at least 100,000 p. s. i., a tensile elongation of at least 2% and a minimum bend ductility of at least 20T.

3. A titanium base alloy consisting essentially of: about 0.5 to 18% antimony; carbon, oxygen and nitrogen up to about 0.6%, 0.4% and 0.3% each, respectively; 0.5 to 40% of at least one beta promoter selected from the group consisting of molybdenum, vanadium, columbium, tantalum, zirconium, manganese, iron, chromium, tungsten, cobalt, nickel, copper, silicon and beryllium, but not to exceed about 25% of chromium and tungsten, 10% of manganese, 7% of iron, 5% of cobalt, nickel and copper, and 2% of silicon and beryllium; 0.25 to 23% of at least one other alpha promoter selected from the group consisting of tin, aluminum, indium, silver, lead and bismuth, but not to exceed 8% aluminum and 15% in total amount of indium, silver, lead and bismuth; the balance of said alloy being substantially titanium, and said alloy being characterized by a tensile strength of at least 100,000 p. s. i., a tensile elongation of at least 2%, and a minimum bend ductility of at least 20T.

4. A titanium base alloy consisting essentially of: about 1 to 18% antimony about 0.5 to 40% of at least one beta-promoting element selected from the group consisting of molybdenum, vanadium, columbium, zirconium and tantalum, carbon up to about 0.6%, oxygen up to about 0.4%, nitrogen up to about 0.3%, characterized in having a beta-containing microstructure, a minimum bend ductility of not over 20T, and an ultimate strength at least 10% in excess of the titanium-base metal.

5. A titanium base alloy consisting essentially of: from more than 5 to about 18% antimony and about 0.25 to 5% aluminum in which the maximum antimony content is related to the aluminum content as follows:

| Percent Aluminum | Maximum Percent Antimony |
|------------------|--------------------------|
| 0.25             | 18                       |
| 1                | 16                       |
| 2                | 14                       |
| 3                | 12.5                     |
| 4                | 11                       |
| 5                | 10                       |

said alloy containing up to about 0.6% carbon, up to about 0.4% oxygen, up to about 0.3% nitrogen, characterized in having a minimum bend ductility not over 20T, and an ultimate strength at least 10% in excess of the unalloyed titanium-base metal.

6. A titanium base alloy consisting essentially of: about 1 to 18% antimony, carbon up to about 0.6%, oxygen up to about 0.4%, nitrogen up to about 0.3%, about 1 to

23% of at least one other alpha-promoting element including aluminum under 3.5%, characterized in having a minimum bend ductility of not over 20T and an ultimate strength at least 10% in excess of the unalloyed titanium-base metal.

7. An alloy consisting of: about 1 to 18% antimony, up to about 0.6% carbon, up to about 0.4% oxygen, up to about 0.3% nitrogen, balance titanium.

8. A titanium base alloy consisting essentially of: about 1 to 18% antimony, up to about 0.6% carbon, up to about 0.4% oxygen, up to about 0.3% nitrogen, under 3.5% aluminum, up to about 22% tin, the maximum tin content being related to the antimony content in accordance with the following tabulation:

| Percent Sb | Percent Sn Max. |
|------------|-----------------|
| 0.5        | 22.5            |
| 5          | 17.5            |
| 10         | 12.5            |
| 15         | 5               |
| 18         | 0               |

said alloy being characterized in having a minimum bend ductility not over 20T, and a tensile elongation of at least 2%.

9. A titanium base alloy consisting essentially of: about 1 to 18% antimony, up to about 0.6% carbon, up to about 0.4% oxygen, up to about 0.3% nitrogen, about 0.5 to 20% of metal selected from the group consisting of chromium and tungsten, characterized in having a minimum bend ductility not over 20T, and an ultimate strength at least 10% in excess of the unalloyed titanium-base metal.

10. A titanium base alloy consisting essentially of: about 1 to 18% antimony, up to about 0.6% carbon, up to about 0.4% oxygen, up to about 0.3% nitrogen, about 0.5 to 10% manganese, characterized in having a minimum bend ductility not over 20T, and an ultimate strength at least 10% in excess of the unalloyed titanium-base metal.

11. A titanium base alloy consisting essentially of: about 1 to 18% antimony, up to about 0.6% carbon, up to about 0.4% oxygen, up to about 0.3% nitrogen, about 0.5 to 7.5% iron, characterized in having a minimum bend ductility not over 20T, and an ultimate strength at least 10% in excess of the unalloyed titanium-base metal.

12. A titanium base alloy consisting essentially of: about 1 to 18% antimony, up to about 0.6% carbon, up to about 0.4% oxygen, up to about 0.3% nitrogen, about 0.5 to 5% of metal selected from the group consisting of copper, nickel and cobalt, characterized in having a minimum bend ductility not over 20T, and an ultimate strength at least 10% in excess of the unalloyed titanium-base metal.

#### References Cited in the file of this patent

#### UNITED STATES PATENTS

- 60 2,554,031 Jaffee ----- May 22, 1951  
 2,596,487 Jaffee ----- May 13, 1952  
 2,669,514 Finlay ----- Feb. 16, 1954

#### OTHER REFERENCES

- 65 Journal of Metals, March 1950, pages 498-499.